

## UNITED STATES PATENT OFFICE

2,668,112

## MANUFACTURE OF PHOTOGRAPHIC COLOR IMAGES

Arthur Henri de Cat, Kessel-Loo, Louvain, Gerard Michiel Stevens, Berchem-Antwerp, and André Emile Van Dormael, Heverlee-Louvain, Belgium, assignors to Gevaert Photo-Producten N. V., Mortsel, Belgium, a company of Belgium

No Drawing. Application December 15, 1951,  
Serial No. 261,932

Claims priority, application Belgium  
December 20, 1950

13 Claims. (Cl. 95—6)

1

This invention relates to a process for the manufacture of photographic color images by color development in the presence of a color coupler, to photographic developers which contain such color couplers, to photographic material which contains such color couplers, and to photographic images obtained according to the process referred to.

It is known to obtain a photographic color image by developing a reducible silver salt image in the presence of a color coupler, i. e., a compound which during development couples with the oxidation product of the developing agent and forms a dyestuff that precipitates onto the developed silver grains.

Yellow and magenta color images are usually obtained by development in the presence of compounds which contain an active methylene group, for instance, compounds wherein the methylene group is connected at one side to a heterocyclic ring and at the other side to another group capable of activating a methylene group, such as, a cyan- or a carbonyl group.

In this class we now have found new color couplers which on color development yield dyestuffs having a favorable absorption for color photography.

It is an object of the present invention to provide a new process for the production of a photographic color image.

It is another object of the present invention to provide a photographic developing solution containing a new class of color couplers.

It is a further object of the present invention to provide a photographic material containing a new class of color couplers.

Further objects of the present invention will appear from the following description.

According to the present invention, a reducible silver salt image is developed with a primary amino aromatic developing agent in the presence of a compound according to the following formula:

(I)



or one of its tautomeric forms, wherein Z is arylene, —CO—R is an acyl-, an ester-, an amide-, a hydrazide- or a hydroxamic acid group.

A tautomeric form of Formula I is, for instance, that wherein the —CO—NH— group is replaced by —C(OH)=N—.

These compounds may be obtained either by

2

causing anthranilic acid or a derivative thereof to react with the imino ether of cyan acetic ester, analogously with the method described by A. Finger and L. Schupp in J. Pr. Chem. (2) 74 (1906) 154, or by effecting a ring closure in an anthranilic acid or -amide, wherein the amino group is substituted by R.CO.CH<sub>2</sub>.CO—, R.CO— having the same significance as indicated hereinbefore, in analogy with the method described by Tomisk and Christensen in J. Am. Chem. Soc. 70 (1948) 1701-2.

The presence of the color couplers according to our invention during color development may arise from the adding to the photographic material, or to the developer, a compound which differs from the color coupler only insomuch as in the active CH<sub>2</sub>- group one or two hydrogen atoms are replaced by a group splitting off either before or during the color development.

20 Our new color couplers may be added to the developer or to a colloid layer, a light-sensitive layer or a non-light-sensitive layer, adjacent to the sensitive layer or separated therefrom by a permeable colloid layer.

25 On color development, some of the new color couplers yield dyestuffs having an absorption as is desired for the use as yellow dyestuff in three-color photography.

The aromatic amino compounds, which according to our invention are added to the developer, comprise the mono-, di- and triamino aryl compound. As mono-amino developers may be mentioned amino-phenols and amino-cresols and their halogen derivatives, and also amino naphthols.

30 The developers preferred for our purposes are the aromatic ortho- and paradiamines, such as, paraphenylenediamines and their substitution products.

35 The following examples serve to illustrate the invention without limiting, however, the scope thereof.

*Example 1*

40 7.95 g. imino ether of cyan acetic acid ethyl ester and 6.85 g. anthranilic acid are refluxed for 5 hours in 30 ccm. alcohol. After cooling, the precipitate formed is sucked off and recrystallized from ethanol. The 2-carbethoxymethyl-4-quinazolone thus obtained corresponds to the following formula:

(II)



45

Melting point: 163° C.

## 3

A photographic film strip is developed in a bath of the following composition:

(A)  
 N:N-diethyl-p-phenylene diamine hydrochloride ----- g. 2  
 Sodium sulphite (cryst.) ----- g. 25  
 Sodium carbonate (cryst.) ----- g. 60  
 Sodium hydroxide ----- g. 2  
 Water to 1000 ccm.

(B)  
 Quinazolone derivative according to Formula II ----- g. 3  
 CH<sub>3</sub>OH or acetone ----- ccm. 1000

For use, (B) is added to (A) while stirring. The developed image is rinsed for 30 minutes and the silver is removed in the following bath:

Potassium ferricyanide ----- g. 50  
 Potassium bromide ----- g. 3  
 Water to 1000 ccm.

The image is again rinsed for 10 minutes and then fixed for 20 minutes in the following bath:

Sodium thiosulphate ----- g. 250  
 Water to 1000 ccm.

and again rinsed for 30 minutes. An intense yellow image with an absorption maximum at about 450 m $\mu$  is obtained.

## Example 2

To 4.4 g. of the compound according to Formula II, dissolved in 100 ccm. alcohol, 0.6 g. hydrazine dissolved in a minimum of alcohol are added. The mixture is boiled for 1 hour on the water bath and the precipitate formed is recrystallized and washed with ethanol. The product obtained corresponds to the following formula:



Melting point: 260° C.

When treating an exposed photographic film strip as is done in Example 1, whereby in the composition (B) the quinazolone derivative according to Formula II is replaced by the derivative according to Formula III, a yellow image is obtained.

## Example 3

2.78 g. hydroxylamine hydrochloride and 0.92 g. sodium are dissolved in 50 ccm. pure alcohol, and 4.6 g. of the compound according to Formula II are added. This mixture is heated for 1 hour on the water bath. After cooling, a precipitate is formed which is washed with ethanol. The hydroxamic acid obtained corresponds to the following formula:



Melting point: 205-210° C.

When treating an exposed photographic film strip as is done in Example 1, whereby in the composition (B) the quinazolone derivative according to Formula II is replaced by the derivative according to Formula IV, an intense yellow image is obtained.

## 4

## Example 4

10 g. 4-nitro-anthranilic acid and 12 g. imino ether of cyan acetic acid ethyl ester are melted together at 60° C. for 4 hours on the water bath. The product obtained is recrystallized from methanol and corresponds to the following formula:



Melting point: 165-168° C.

When treating an exposed photographic film strip as is done in Example 1, whereby in the composition (B) the quinazolone derivative according to Formula II is replaced by the derivative according to Formula V, an orange image with an absorption maximum at 465 m $\mu$  is obtained.

## Example 5

The compound according to Formula V is dissolved in ethanol and catalytically reduced under 1 to 2 atmosphere pressure with Raney nickel. After evaporation of the alcohol, the amino derivative according to the following formula:



is obtained.

Melting point: 180-185° C.

When treating an exposed photographic film strip as is done in Example 1, whereby in the composition (B) the quinazolone derivative according to Formula II is replaced by the derivative according to Formula VI, an intense yellow image with an absorption maximum at 450 m $\mu$  is obtained.

## Example 6

To 3.4 g. anthranil amide dissolved in 10 ccm. chloroform are added 2.1 g. diketene. The mixture is heated until a homogeneous solution is obtained. This solution is left for 24 hours at room temperature whereafter the precipitate formed is sucked off. After recrystallization from ethanol, aceto-acethyl anthranil amide is obtained. Melting point: 142-144° C. 5.5 g. of the product obtained are dissolved in 10 ccm. aqueous solution of NaOH 5%. The solution is heated on the water bath for 40 minutes and neutralized with acetic acid to pH 7. The precipitate formed is sucked off and recrystallized from dioxane. The compound obtained corresponds to the following formula:



Melting point: 212-213° C.

When treating an exposed photographic film strip as is done in Example 1, whereby in the composition (B) the quinazolone derivative according to Formula II is replaced by the derivative according to Formula VII, an intense yellow image is obtained.

## Example 7

2.05 g. imino ether of para-methyl cyanaceto-

phenone and 1.33 g. anthranilic acid are heated together on the boiling water bath. After 20 minutes, the mass melts but heating is continued for 5 more hours. The precipitate formed is recrystallized from glycol-monomethyl ether. The product obtained corresponds to the following formula:

(VIII)



Melting point: above 250° C.

When treating an exposed photographic film strip as is done in Example 1, whereby in the composition (B) the quinazolone derivative according to Formula II is replaced by the derivative according to Formula VIII, an intense yellow image is obtained.

*Example 8*

3.6 g. imino ether of furoyl acetonitrile and 2.74 g. anthranilic acid are melted together on the boiling water bath and then heated for 3 hours. The oil obtained is shaken with an aqueous solution of Na<sub>2</sub>CO<sub>3</sub> and the solution obtained is acidified with acetic acid. The precipitate formed is sucked off. The compound obtained corresponds to the following formula:

(IX)



Melting point: above 250° C.

When treating an exposed photographic film strip as is done in Example 1, whereby in the composition (B) the quinazolone derivative according to Formula II is replaced by the derivative according to Formula IX, an intense yellow-orange image is obtained.

*Example 9*

1.87 g. 2-amino-1-naphthoic acid and 2.40 g. imino ether of cyan acetic acid ethyl ester are heated together for 2 hours at 60° C. on the water bath. The solid product formed is recrystallized from dioxane. Melting point: 183-185° C. The compound obtained corresponds to the following formula:

(X)



When treating an exposed photographic film strip as is done in Example 1, whereby in the composition (B) the quinazolone derivative according to Formula II is replaced by the derivative according to Formula X, an intense yellow image is obtained.

*Example 10*

2.18 g. quinazolonyl acethydrazide according to Formula III and 3.24 g. hexadecyl succinic acid anhydride are refluxed for 3 hours in 20 ccm. dioxane. After cooling, the precipitate formed is separated by filtration and purified by dissolving in an aqueous solution of NaOH 2N and precipitating with an aqueous solution of HCl 2N. After recrystallization from dioxane, the melting

point is 168-170° C. The compound obtained corresponds to the following formula:

(XI)



1 g. of this product is dissolved in 15 ccm. of 10 a 1/2 N aqueous solution of NaOH. Water is added until the volume of the solution reaches 25 ccm. This solution is added to 100 ccm. of an emulsion for positive ciné film. This emulsion is coated onto a film support, exposed and developed in the following bath:

N,N-diethyl - p - phenylene-diamine hydrochloride ----- g. 5  
Sodium sulphite (cryst.) ----- g. 10  
20 Sodium carbonate (cryst.) ----- g. 100  
Sodium hydroxide ----- g. 1  
Water to 1000 ccm.

washed, bleached in order to remove the silver, and fixed as in Example 1. A yellow-orange 25 image is obtained.

We claim:

1. Process for the production of a photographic color image by developing a reducible silver salt image with a primary amino aromatic developing agent in the presence of a color coupler corresponding to the following formula:

35



wherein Z is arylene, —CO—R is a member selected from the group consisting of an acyl-, an ester-, an amide-, a hydrazide- and a hydroxamic acid group.

2. Process for the production of a photographic color image by developing a reducible silver salt image with a developing solution containing a primary amino aromatic developing agent and a color coupler corresponding to the following formula:

50



wherein Z is arylene, —CO—R is a member selected from the group consisting of an acyl-, an ester-, and amide-, a hydrazide- and a hydroxamic acid group.

3. Process for the production of a photographic color image by developing with a primary amino aromatic developing agent a reducible silver salt image in a photographic material containing a color coupler corresponding to the following formula:

65



70 wherein Z is arylene, —CO—R is a member selected from the group consisting of an acyl-, an ester-, an amide-, a hydrazide- and a hydroxamic acid group.

4. Photographic developer containing a primary amino aromatic developing agent and a col-

or coupler corresponding to the following formula:



wherein Z is arylene, —CO—R is a member selected from the group consisting of an acyl-, an ester-, an amide-, a hydrazide- and a hydroxamic acid group.

5. Light-sensitive photographic material comprising a silver halide emulsion layer and a color coupler corresponding to the following formula:



wherein Z is arylene, —CO—R is a member selected from the group consisting of an acyl-, an ester-, an amide-, a hydrazide- and a hydroxamic acid group.

6. Photographic developer containing a primary amino aromatic developing agent and a color coupler corresponding to the following formula:



wherein Z is arylene, —CO—R is acyl.

7. Photographic developer containing a primary amino aromatic developing agent and a color coupler corresponding to the following formula:



wherein Z is arylene, —CO—R is a hydrazide group.

8. Light-sensitive photographic material comprising a silver halide emulsion layer and a compound corresponding to the following formula:



wherein Z is arylene, —CO—R is a hydrazide group.

9. Photographic developer containing a primary amino aromatic developing agent and a compound having the following formula:



10. Photographic developer containing a primary amino aromatic developing agent and a compound having the following formula:



11. Photographic developer containing a primary amino aromatic developing agent and a compound having the following formula:



12. Photographic developer containing a primary amino aromatic developing agent and a compound having the following formula:



13. Light-sensitive photographic material comprising a silver halide emulsion layer and a compound having the following formula:



ARTHUR HENRI DE CAT.  
GERARD MICHAEL SEVENS.  
ANDRÉ EMILE VAN DORMAEL.

References Cited in the file of this patent

UNITED STATES PATENTS

| Number    | Name                  | Date          |
|-----------|-----------------------|---------------|
| 2,396,917 | Hanford et al. _____  | Mar. 19, 1946 |
| 2,408,633 | Guenther et al. _____ | Oct. 1, 1946  |